# EUROPEAN PATENT SPECIFICATION

(11) **EP 2 619 628 B1**
(45) Date of publication and mention of the grant of the patent: **26.03.2014**
(21) Application number: 11758544.8
(22) Date of filing: 07.09.2011
(51) Int. Cl.: G03C 1/95

(54) **PHOTOGRAPHIC PAPER AND ITS USE IN A PHOTO ALBUM**
PHOTOGRAPHISCHES PAPIER UND SEIN GEBRAUCH IN EIN PHOTOALBUM
PAPIER PHOTOGRAPHIQUE ET SON EMPLOI DANS UN ALBUM PHOTOGRAPHIQUE

(30) Priority: 20.04.2011 GB 201106658; 17.09.2010 US 383917 P; 17.09.2010 GB 201015575
(43) Date of publication of application: 31.07.2013
(73) Proprietor: Fujifilm Manufacturing Europe BV, 5047 TK Tilburg (NL)
(72) Inventor: DE MUNNIK, Mattijs, NL-5047 TK Tilburg (NL); VAN KESSEL, Petrus, NL-5047 TK Tilburg (NL)
(74) Representative: Mayall, John
(86) International application number: PCT/GB2011/051668
(87) International publication number: WO 2012/035314

(56) References cited:
- EP-A1- 0 726 490
- EP-A2- 0 019 178
- DE-A- 2 758 767
- GB-A- 1 483 551
- GB-A- 2 368 653
- JP-A- 2003 114 501
- JP-A- 2003 215 742
- JP-A- 2009 020 350
- US-A- 4 190 449

## Description

This invention relates to a photographic paper, its preparation and use for making album-books.

Typically photographic paper comprises a base layer coated with one or more layers of light-sensitive chemicals. For colour photography, the paper will typically comprise three light-sensitive emulsion layers (yellow, magenta and cyan) to provide a full colour image, optionally with other layers.

During manufacture and storage, photographic papers can suffer from the problem of sticking together, due to the inherent stickiness of their outer-most layer.

In use, photographic paper is exposed to light in a controlled manner to generate an image whereon, for example using an image obtained on a camera film or using a digital image. The desired image then develops and the resultant photographic paper carrying the desired image is often referred to as a photograph. The photograph may be stacked along with other photographs, 'back-to-back', and handed or posted to the photographer. Thereafter, it is quite common for the photograph (i.e. the photographic paper carrying the desired image) to be included in an album-book where the photographs contact each other in a 'face-to-face' manner as a result of being on opposite pages. This 'face-to-face' contact can cause problems, particularly when the album-book is stored under hot and/or humid conditions. The photographs are prone to sticking together, causing them damage when pages of the album-book are opened, sometimes spoiling irreplaceable family pictures.

One method for preventing photographs from sticking to each other in album books is to place an interfoil of light paper as a barrier between the photographs. However this makes the album more expensive, the interfoil is prone to damage and it interferes with the easy viewing of two open pages at once. It is also possible for photographs to stick to the interfoil.

The present invention seeks to address the problem of photographic paper sticking together, whether it be during manufacture or storage of the unused photographic papers or whether it be photographic paper carrying images stored in album-books or other environments.

GB 1,483,551, Example 1, describes the application of a protective layer to a cellulose triacetate photographic film of the kind loaded into conventional, non-digital cameras. The protective layer for the film may include gelatin and colloidal silica having a mean particle size of 20 nm.

According to the present invention there is provided photographic paper comprising an outer-most layer comprising a hydrophilic colloid binder and colloidal silica, wherein:
(i) the weight ratio of colloidal silica to hydrophilic colloid binder in said layer is 0.3:1 to 3:1; and
(ii) the colloidal silica has a mean particle size of 2 to 10 nm.

The components of the photographic paper depend to some extent on whether an image has been developed thereon, i.e. whether or not the photographic paper has been used. Before an image is developed on the photographic paper, it typically comprises a base layer (e.g. polyester or resin-coated paper), one or more light-sensitive emulsion layers (e.g. layers which generate yellow, magenta or cyan colours) and the aforementioned outer-most layer on top of the one or more light-sensitive emulsion layers. After an image has been developed, the photographic paper typically comprises the same components except that the light-sensitive layers are no longer light sensitive, having been exposed to light in a controlled manner to develop the desired image thereon.

Preferably the colloidal silica has a mean particle size of 3 to 9 nm, especially 4 to 9 nm. This preference arises because colloidal silica having a mean particle size below 2 nm can increase the viscosity of coating solutions, leading to longer manufacturing times for the photographic paper or the requirement for expensive viscosity reducing agents to be included in coating compositions.

Preferably the outer-most layer comprises 0.3 g/m² to 1.5. g/m², more preferably 0.7 g/m² to 1.15 g/m², especially about 0.86 g/m² of the colloidal silica.

The photographic papers of the present invention have excellent anti-sticking properties and may be prepared conveniently at high speeds above 200 m/min using, for example, a slide coater or a curtain coater.

As the function of the outer-most layer of the present invention is to prevent the image receiving surface of photographic paper from sticking to other surfaces, the outer-most layer generally does not include any silver halide.

The colloidal silica preferably consists essentially of silicon dioxide. Optionally the colloidal silica may contain, as a minor component, alumina or sodium aluminate, e.g. in an amount of 0 to 0.1 g per g of the silicon dioxide. The colloidal silica optionally comprises, as a stabilizer, an inorganic base, for example sodium hydroxide, potassium hydroxide, lithium hydroxide or ammonia, or an organic base such as a tetraethylammonium salt.

The colloidal silica can be employed in the form of a colloidal dispersion of fine particles of silica in a medium such as water or an organic liquid, for example, methanol, ethanol, propanol, butanol, acetone, ethyl acetate or butyl acetate.

Preferred in this invention is the use of silicate sol or silicic acid sol in a water environment. However the weight of other components (e.g. water, organic liquid etc.) are not taken into account when calculating the weight ratio of colloidal silica to hydrophilic colloid binder.

Examples of commercially available products comprising colloidal silica include Levasil^{™} 300 and Levasil^{™} 500 from H.C. Starck. According to the manufacturer's catalogue these products contain colloidal silica having mean particle sizes of 9 nm and 6 nm respectively and surface areas of 300 g/m² and 450 g/m² respectively. Also Bindzil^{™} 30/360 may be used (7 nm). Other commercially available colloidal silicas include NexSil^{™} 5 (6 nm) and NexSil^{™} 8 (8 nm) from Nyacol Nano Technologies, Inc. The colloidal silicas may be surface-treated if desired.

In our experiments the inclusion of colloidal silica having a mean particle size above 10 nm in the outer-most layer did not result in any improvement in anti-sticking property for the resultant substrate.

The anti-sticking property of photographic papers is extremely important for glossy colour photographic papers intended for storage in album-books. In the absence of an anti-sticking layer according to the present invention, the photographs facing each other tend to stick together and need to separating using high forces which can result in damage to the photograph and/or a dulling of the appearance of the photographs.

Preferably the weight ratio of colloidal silica to hydrophilic colloid binder in said outer-most layer is 0.3:1 to 2:1.

We have found that when the outer-most layer comprises 0.3 to 1.5 g/m² of colloidal silica and the weight ratio of colloidal silica to hydrophilic colloid binder is 0.3:1 to 3:1 (preferably 0.3:1 to 2:1) the photographic papers demonstrate particularly good anti-stick properties without detracting from the physical appearance of the images they carry. Furthermore, the viscosity of compositions required to provide colloidal silica loadings of 1.5 g/m² or less of and a ratio of colloidal silica to hydrophilic colloid binder of 3:1 or less (preferably 2:1 or less) are generally low enough at high shear rates to be applied to a base layer carrying one or more light-sensitive emulsion layers in one step in a multi-layer coating method, e.g. at speeds higher than 150 m/min using a slide coater or curtain coater. Speeds higher than 200 m/min (i.e. for example 300 m/min or 350 m/min) may even be achieved. When the ratio of colloidal silica to hydrophilic colloid binder is lower than 0.3 the anti-stick effect is sometimes inadequate.

The photographic papers of the present invention also have good writability. In other words, the papers are receptive to subsequent marking with ink and even with pencil. The hydrophilic colloid binder preferably is or comprises a gelatin. Preferred gelatins include acid-processed gelatin, mixtures comprising acid-processed gelatin and alkali-processed gelatin and optionally other hydrophilic binders.

Preferred acid-processed gelatins include gelatins produced by treating collagen with hydrochloric acid, etc., and differ from the typical alkali-processed gelatins used in the photographic industry. Details of the processes for producing acid- and alkali-processed gelatins and the properties thereof are described in Arthur Veis, The Macromolecular Chemistry of Gelatin, pages 187-217, Academic Press (1964). Preferred acid-processed gelatins have an isoelectric point at a pH of about 6.0 to 9.5, whereas alkali-processed gelatin typically have an isoelectric point at a pH of about 4.5 to 5.3.

The hydrophilic colloid binder preferably comprises an acid-processed gelatin and a further hydrophilic binder other than an acid-processed gelatin, e.g. an alkali-processed gelatin, an enzyme-processed gelatin or a gelatin derivative. Gelatin derivatives may be prepared by treating and modifying the functional groups contained in the gelatin molecule with chemicals other than simple acids and alkalis. For example, amino groups, imino groups, hydroxyl groups or carboxyl groups normally present in gelatin may be reacted with a compound having a group capable of reacting with such a functional group. One may also graft a polymer or another high molecular weight material to gelatin in order to make a gelatin derivative. Compounds having groups capable of reacting the functional groups in gelatin include, for example, isocyanates, acid chlorides and acid anhydrides, e.g. as described in US 2,614,928; acid anhydrides as described in US 3,118,766; bromoacetic acids; phenylglycidyl ethers; vinylsulfone compounds, e.g. as described in US 3,132,945; N-allylvinylsulfonamides, e.g. as described in GB 861,414; maleinimide compounds, e.g. as described in US 3,186,846; acrylonitriles, e.g. as described in US 2,594,293; polyalkylene oxides, e.g. as described in US 3,312,553; epoxy compounds; acid esters, e.g. as described in US 2,763,639; alkane sulphones, e.g. as described in GB 1,033,189.

In addition, suitable hydrophilic colloid binders include proteins, e.g. colloidal albumin and casein; cellulose derivatives, e.g. carboxymethyl cellulose and hydroxyethyl cellulose; polysaccharides, e.g. agar-agar, sodium alginate, dextran, gum arabic and starch derivatives; and synthetic hydrophilic colloids, e.g. polyvinyl alcohol, poly-N-vinylpyrrolidone, polyacrylic acid copolymer, polymethacrylic acid copolymer, polyacrylamide and polymethacrylamide; and mixures and derivatives thereof. If desired, a compatible mixture comprising two or more of these hydrophilic colloid binders can be used. Of the above-described hydrophilic colloid binders, gelatin derivatives and synthetic high molecular weight materials having carboxyl group or salt thereof are particularly preferred. There are no particular restrictions on the mixing ratio of acid to processed gelatin and the above-described other hydrophilic colloid binders, but in order to obtain particularly good results, the hydrophilic colloid binder preferably comprises at least 20 wt%, more preferably at least 40 wt% acid-processed gelatin. When the hydrophilic colloid binder comprises at least 20 wt% of acid-processed gelatin is less than about 20 wt%, and alkali-processed gelatin, enzyme-processed gelatin or a gelatin derivative is not present as part of the hydrophilic colloid binder, compositions used to apply the outer-most layer to the substrate set (solidify) particularly well, improving the likelihood that a uniform and smoothly coated surface will result.

The said outer-most layer preferably comprises 0.2 to 1.5 g/m² of hydrophilic colloid binder.

The photographic paper of the present invention preferably comprises 4 to 8 g/m², preferably 5 to 7 g/m², of hydrophilic colloid binder.

Optionally the outer-most layer comprises one or more further ingredients, for example a matting agent, hardening agent, lubricant, surface active agent and/or or pH-regulator.

Examples of suitable matting agents include certain organic compounds, e.g. water-dispersible vinyl polymers, e.g. polymethylacrylate, polymethylmethacrylate and/or polystyrene, and certain inorganic compounds, e.g. silver halide, strontium barium sulphate, magnesium oxide and/or titanium oxide.

In an especially preferred in an embodiment the outer-most layer further comprises polymethyl methacrylate (PMMA), especially PMMA having a mean size of 3 to 10 microns (e.g. 4 microns), preferably in an amount of 2 to 50 mg/m² (e.g. 10 mg/m²)_{.}

As lubricants one may use, for example, a wax, liquid paraffin, a higher fatty acid esters, a polyfluorinated hydrocarbon or derivative thereof, a silicone such as polyalkylpolysiloxane, polyarylsiloxane, polyalkylarylpolysiloxane and/or an alkyleneoxide adduct thereof.

In one embodiment the outer-most layer comprises one or more hardening agents. Such hardening agents may be included to enhance the physical strength of a outer-most layer. Specific examples of suitable hardening agents include aldehyde compounds, e.g. formaldehyde and glutaraldehyde; ketone compounds, e.g. diacetyl and cyclopentanedione; compounds containing reactive halogens, e.g. bis(2-chloroethylurea) and 2-hydroxy-4,6-dichloro-1,3,5-triazine; the compounds described in US 3,288,775, US 2,732,303, GB 974,723 and GB 1,167,207; reactive olefin compounds, e.g. divinyl sulfone, 5-acetyl-1,3-diacryloylhexahydro-1,3,5-triazine and the compounds described in US 3,635,718, US 3,232,763 and GB 994,869; N-methylol compounds, e.g. N-hydroxymethylphthalimide and compounds described in US 2,732,316 and US 2,586,168; isocyanates, e.g. as described in US 3,103,437; aziridine compounds, e.g. as described in US 3,017,280 and US 2,983,611; the acid derivatives described in US 2,725,294 and US 2,725,295; carbodiimide compounds, e.g. as described in US 3,100,704; epoxy compounds, e.g. as described in US 3,091,537; isooxazole compounds, e.g. as described in US 3,321,313 and US 3,543,292; halocarboxyaldehydes, e.g. mucochloric acid; dioxane derivatives, e.g. dihydroxydioxane and dichlorodioxane; and inorganic hardening agents, e.g. chrome alum and zirconium sulfate. Moreover, in place of the above compounds, hardening agent precursors such as alkali metal bisulfite-aldehyde adducts, methylol derivatives of hydantoin and primary aliphatic nitroalcohols can be used. A particularly preferred hardening agent is 1-oxy-3,5-dichloro-s-triazine and salts thereof, e.g. the sodium salt.

It is preferred that the ratio (R) of hardening agent to hydrophilic colloid binder in said outer most layer satisfies the following equation: $R = \left(Hmol/HCg\right)$
wherein:
- R: is greater than 0.00013;
- Hmol: is the number of moles of hardening agent; and
- HCg: is the weight in grams of hydrophilic colloid binder.

The above preference for R is particularly so when the outer-most layer comprises a hardening agent. While the above preference is expressed in terms of the outer-most layer, there is also a preference for the photographic paper as a whole (i.e. not just the outer-most layer) to have a ratio (R) of hardening agent to hydrophilic colloid binder as defined above.

In the above equation, the weight of hydrophilic colloid binder is in grams on a 100% solids basis. For example, when the hydrophilic colloid binder is a gelatin, as is preferred, the weight of any water present in the binder is not included when calculating the weight of hydrophilic colloid binder in grams. One may calculate the weight of hydrophilic colloid binder on a 100% solids basis by, for example, drying it to remove any water or organic solvents to find its strength and multiplying the strength against the amount used.

Preferably R has a value of 0.00014 to 0.00018.

When R has the values mentioned above the resultant photographic paper will often benefit from an improved ability to peel-apart from another sheet of photographic paper, without significantly damaging images, after being stored together in a face-to-face manner. We refer to this as "improved peeling behaviour".

Surface active agents can also be included in the outer-most layer, individually or as a mixture thereof, e.g., in an amount of from about 0.5 to 50 mg, preferably 1 to 20 mg, per g of hydrophilic colloidal binder. They are generally used as a coating aid for preventing the occurrence of difficulties such as unevenness in coating, but they are sometimes employed for other purposes, for example, for improving emulsification and dispersion, for preventing the formation of static charges. These surface active agents can be classified as natural surface active agents, e.g. such as saponin; nonionic surface active agents; e.g. such as alkylene oxide, glycerol and glycidol nonionic surface active agents; cationic surface active agents, e.g. such as higher alkylamines, quaternary ammonium salts, pyridinium and other heterocyclic onium salts, phosphoniums and sulfoniums; anionic surface active agents containing acid groups, e.g. such as carboxylic acid, sulfonic acid, phosphoric acid, sulfuric ester or phosphoric ester groups; and amphoteric surface active agents, e.g. such as amino acids, aminosulfonic acids, or sulfuric or phosphoric esters of aminoalcohols.

The surface active agents which can be used are described in, for example, US 2,271,623, 2,240,472, 3,441,413, 3,442,654, 3,475,174 and 3,545,974, German Patent Application (OLS) No. 1,942,665 and GB 1,077,317 and GB 1,198,450, as well as in Ryohei Oda et al., Synthesis and Applications of Surface Active Agents, Maki Publisher (1964), A.M. Schwartz et al., Surface Active Agents, Interscience Publications In. (1958), and J.P. Sisley et al., Encyclopedia of Surface Active Agents, Vol. 2, Chemical Publishing Company (1964).

The photographic paper of this invention optionally contains the following components and can be prepared by the production methods described below.

Silver halide emulsions for light-sensitive emulsion layer(s) are usually prepared by mixing a solution of a water-soluble silver salt (such as silver nitrate) with a solution of a water-soluble halide (such as potassium bromide or sodium chloride) in the presence of a solution of a water-soluble high molecular weight material such as gelatin. Silver halides which can be used include silver chloride, silver bromide, as well as mixed silver halides such as silver chlorobromide, silver bromoiodide or silver chlorobromoiodide. The silver halide grains can be prepared using conventional methods. Of course, the grains can be advantageously prepared using the so-called singe or double jet method, controlled double jet method. Moreover, two or more of silver halide photographic emulsions, separately prepared, can be mixed, if desired.

The crystal structure of the silver halide grains can optionally be uniform throughout the grain, can have a stratified structure in which the interior and outer portion are different, or can be of the so-called conversion type as described in GB 635,841 and US 622,318. In addition, the silver halides can be of the type in which a latent image is formed mainly on the surface of the grains or of the type in which a latent image is formed in the interior of the grains thereof.

The above photographic emulsions are described, e.g., in C.E.K. Mees & T.H. James, The Theory of the Photographic Process, 3rd Ed., Macmillan, New York (1966); P. Glafkides, Chimie et Physique Photographiques, Paul Montel, Paris (1957); etc., and can be prepared using various methods which are usually employed such as an ammonia process, a neutral process or an acid process.

Especially preferred are the silver halide grains as prepared and described in US 6,949,334.

The silver halide grains may, after the formation thereof, be washed with water to remove the water-soluble salts produced as by-products (for example, potassium nitrate when silver bromide is prepared using silver nitrate and potassium bromide) from the system and then heat treated in the presence of a chemical sensitizer such as sodium thiosulfate, N,N,N'-trimethylthiourea, gold(I) thiocyanate complex, gold(I) thiosulfate complex, stannous chloride or hexamethylenetetramine to increase the sensitivity without coarsening the grains. Conventional sensitizing methods are described in Mees and James, supra, and Glafkides, supra,

Hydrophilic colloids which can be used as a vehicle for silver halide include gelatin, colloidal albumin, casein, cellulose derivatives such as carboxymethyl cellulose or hydroxyethyl cellulose, polysaccharides such as agar-agar, sodium alginate or starch derivatives, and synthetic hydrophilic colloids such as polyvinyl alcohol, poly-N-vinylpyrrolidone, polyacrylic acid copolymers or polyacrylamide, and the derivatives thereof and the partially hydrolyzed products thereof. If desired, a compatible mixture of two or more of these hydrophilic colloids can be used. Of the above-described hydrophilic colloids, gelatin is most generally used, but gelatin can be, partially or completely, replaced with a synthetic high molecular weight material. Furthermore, the gelatin can be replaced with a so-called gelatin derivative, e.g. as described above.

In the photographic emulsion layer(s) and other layers which may be used in this invention, synthetic polymer compounds such as a latex of water-dispersible vinyl compound polymers, particularly, compounds increasing the dimensional stability of the photographic material can be incorporated as such or as a mixture (e.g., of different polymers), or in combination with hydrophilic colloids which are permeable to water. Many such polymers are known, and are described, e.g., in US Pat. Nos. 2,375,005, 3,607,290 and 3,645,740, British Pat. Nos. 1,186,699 and 1,307,373, etc. Of these polymers, copolymers or homopolymers of alkyl acrylates, alkyl methacrylates, acrylic acid, methacrylic acid, sulfoalkyl acrylates, sulfoalkyl methacrylates, glycidyl acrylate, glycidyl methacrylate, hydroxyalkyl acrylates, hydroxyalkyl methacrylates, alkoxyalkyl acrylates, alkoxy methacrylate, styrene, butadiene, vinyl chloride, vinylidene chloride, maleic anhydride and itaconic anhydride are generally used. If desired, the so-called graft-type emulsion-polymerized latices of these vinyl compounds which are prepared by subjecting such a vinyl compound to emulsion polymerization in the presence of a hydrophilic protective colloid high molecular weight material can be used.

The photographic papers of the present invention generally contain one or more light-sensitive, silver halide emulsion layers between the outer-most layer and a base layer. The silver halide emulsion layer(s) can be sensitized in a conventional manner. Suitable chemical sensitizers include, e.g., gold compounds, e.g. such as chloroaurate or auric trichloride as described in US Pat. Nos. 2,399,083, 2,540,085, 2,597,856, 2,597,915 and 6,949,334; salts of noble metals, e.g. such as platinum, palladium, iridium, rhodium or ruthenium as described in US Pat. Nos. 2,448,060, 2,540,086, 2,566,245, 2,566,263, 2,598,079 and 6,949,334 and sulfur compounds capable of forming silver sulfide by reacting with a silver salt, e.g. as described in US Pat. Nos. 1,574,944, 2,410,689, 3,189,458 and 3,501,313; stannous salts, e.g. as described in US Pat. Nos. 2,487,850 and 2,518,698; amines; and other reducing compounds. Preferred techniques are gold sensitization, sulfide and/or Iridium sensitization as described in US 6,949,334 with general formula (i) on page 12. For the gold sensitization, auro (I) complex having various inorganic gold compounds or inorganic ligands, and auro (I) compound having organic ligands can be used if desired.

For the inorganic gold compound, chloroauric acid or the salt thereof can be used for instance. For the auro (I) complex having inorganic ligands, auro dithiocyanate compounds such as potassium auro (I) dithiocyanate and auro dithiosulfate compound such as trisodium auro (I) dithiosulfate can be used, for example.

Further, auro (I) thiolate compound described in US 3,503,749, gold compounds described in JP-A Nos. 8-69074, 8-69075, and 9-269554, US Pat. Nos. 5,620,841, 5,912,112, 5,620,841, 5,939,245 and 5,912,111 can also be used.

Various compounds can be added to the emulsion layer(s) of the photographic paper in order to prevent a reduction in sensitivity and the occurrence of fog during production of the photographic paper, during storage, and during processing. Many such compounds are known, for example, 4-hydroxy-6-methyl-1,3,3a, 7-tetraazaindene, 3-methylbenzothiazole, 1-phenyl-5-mercaptotetrazole, 5-arylamino-1,2,3,4-thiatriazole, as well as a large number of heterocyclic compounds, mercury-containing compounds, mercapto compounds, metal salts. Examples of such compounds which can be used are described in C.E.K. Mees & T.H. James, supra and the original references cited therein, and also in the following patents: US Pat. Nos. 1,758,576, 2,110,178, 2,131,038, 2,173,628 and GB 893,428, 403,789, 1,173,609 and 1,200,188 and EP 447,647. Especially preferred for improving the storability of the silver halide emulsion, the following compounds are preferably used also in the present invention: hydroxamic acid derivatives described in JP-A No. 11-109576, cyclic ketones having double bonds substituted for an amino group or a hydroxyl group on both ends adjacent with a carbonyl group described in JP-A No. 11-327094 (particularly, those represented by the general formula (S1); descriptions in column Nos. 0036 to 0071 can be incorporated in the present specification), sulfo-substituted cathecol or hydroquinones described in JP-A No. 11-143011 (for example, 4,5-dihydroxy-1,3-benzenedisulfonic acid, 2,5-hydroxy 1,4-benzenedisulfonic acid, 3,4-dihydroxybenzenesulfonic acid, 2,3-dihydroxybenzenesulfonic acid, 2,5-dihydroxybenzenesulfonic acid, 3,4,5-trihydroxybenzenesulfonic acid and salts thereof), hydroxylamines represented by the general formula (A) in the specification US Pat. No. 5,556,741 (descriptions in column 4, line 56 to column 11, line 22 of the specification of the US Pat. No. 556,741 can be applied preferably also in the present invention and can be incorporated as a portion of the specification of the present application), and water soluble reducing agents represented by the general formulae (I) to (III) in JP-A No. 11-102045.

The light-sensitive emulsion layer(s) can be, if desired, spectrally sensitized or supersensitized using cyanine dyes such as cyanine, merocyanine or carbocyanine individually or in admixture, or in combination with, e.g., styryl dyes. Such color sensitization techniques are known in the art.

The light-sensitive emulsion layers can be hardened if desired using a hardening agent. Examples of suitable hardening agents are mentioned above.

The emulsion layer(s) optionally contain surface active agents, individually or in admixture.

Preferred base layers include papers. Such papers are optionally coated or laminated with baryta or a polymer of an alpha-olefin, particularly having 2 to 10 carbon atoms, for example, polyethylene, polypropylene, ethylene-butene copolymers, etc., or synthetic resin films the surface of which has been roughened to improve the adhesion to other high molecular weight materials and improve printability. If desired the lamination of the polymer on the paper is done via a multi-layer using a co-extrusion technique having pigment in an intermediate polymer layer.

Preferred base layers are photographic grade base papers, optionally laminated on one or both sides with a polyethylene resin, preferably with a ratio of resin weight of top-side resin to back-side ranging from 0.70:1 to 1.30:1 and even more preferably between 0.85:1 and 1.15:1.

The base layer preferably has a thickness of 100 to 250 microns (e.g. 147 or 160 or 225 microns).

The base layer can be further colored with a dye or a pigment if desired.

If the adhesion between the base layer and the light-sensitive emulsion layer(s) is insufficient, a layer having good adhesion to both of these elements can be employed as a subbing layer. For further improving the adhesive property of the base layer, the surface of the base layer can be subjected to a pre-treatment such as a corona discharge, an ultraviolet irradiation, an ozone treatment, a flame treatment.

The outer-most layer and light-sensitive emulsion layer(s)may be applied to a base layer by any suitable technique, including dip coating, air-knife coating, curtain coating, and extrusion coating. If desired, two or more layers can be coated at the same time using the techniques as described in US Pat. Nos. 2,761,791, 3,508,947, 2,941,898 and 3,526,528.

Preferably the outer-most layer and the underlying light-sensitive emulsion layer(s) are applied to the base layer simultaneously, preferably using a slide coater or curtain coater, preferably at a coating speed higher than 200 m/min.

The photographic papers optionally further comprise an intermediate layer, a filter layer, a subbing layer, an antihalation layer, etc.

The photographic papers of this invention may be developed, after exposure, to form color images, to give what are often referred to as photographs. Development processing may include several steps (for example, a combination of bleaching, fixing, bleach-fixing, stabilizing, washing, etc.) and can be effected at a temperature below about 20°C, or higher temperatures, and, if desired, at above about 30°C, and preferably at about 32°C to 60°C. Again, the steps need not always be effected at the same temperature, and they can be carried out at higher or lower temperatures.

Color developers are alkaline aqueous solutions containing a compound whose oxidized product reacts with a color coupler to form a dye, that is, containing, as a developing agent, p-phenylenediamines such as N,N-diethyl-p-phenylenediamine, N,N-diethy-3-methyl-p-phenylenediamine, 4-amino-3-methyl-N-ethyl-N-methanesulfonamidoethylaniline, 4-amino-3-methyl-N-ethyl-N-.beta.- hydroxyethylaniline and N-ethyl-N-.beta.-hydroxyethyl-p-phenylenediamine, or salts thereof such as the hydrochlorides, sulfates and sulfites thereof. The alkaline aqueous solution has a pH higher than about 8, preferably from 9 to 12. The compounds as described in US Pat. Nos. 2,193,015 and 2,592,364 can also been used as a developing agent. The color developers can contain, in addition to the above developing agent, a salt such as sodium sulfate; a pH modifier such as sodium hydroxide, sodium carbonate or sodium phosphate; a buffer, for example, an acid such as acetic acid or boric acid, or a salt thereof; and a development accelerator, for example, various pyridinium compounds, cationic compounds, potassium nitrate and sodium nitrate as described in US Pat. Nos. 2,648,604 and 3,671,247, polyethylene glycol condensates and the derivatives thereof as described in US Pat. Nos. 2,533,990, 2,577,127 and 2,950,970, nonionic compounds such as polythioethers represented by the compounds as described in British Pat. Nos. 1,020,033 and 1,020,032, polymer compounds containing sulfite ester groups represented by the compounds as described in US 3,068,097, as well as organic amines such as pyridine or ethanolamine, benzyl alcohol, hydrazines, etc. Moreover, the color developers can contain an antifogging agent, for example, alkali metal bromides, alkali metal iodides, nitrobenzimidazoles as described in US Pat. Nos. 2,496,940 and 2,656,271, as well as mercaptobenzimidazole, 5-methylbenztriazole, 1-phenyl-5-mercaptotetrazole, compounds for rapid processing as described in US Pat. Nos. 3,113,864, 3,342,596, 3,295,976, 3,615,522 and 3,597,199, thiosulfonyl compounds as described in GB 972,211, phenazine-N-oxides, antifogging agents as described in Manual of Scientific Photography, Vol. 2, pages 29-47, etc.; a stain- or sludge-preventing agent as described in US Pat. Nos. 3,161,513 and 3,161,514, and British Pat. Nos. 1,030,442, 1,144,481 and 1,251,558; an agent for accelerating the interimage effect as described in US 3,536,487; and an antioxidant such as a sulfite, hydrogen sulfite, hydroxylamine hydrochloride or formaldehyde-alkanolamine sulfite adducts.

All of the additives exemplified for each of the processing steps described above and the amount thereof employed are known in the art of color photographic processing methods.

After color development, the photographic papers are usually bleached and fixed. Bleach and fixation can be combined and, thus, a bleach-fix bath can be used. Many compounds can be used as a bleaching agent, but of these compounds, generally ferricyanide salts, dichromate salts, water-soluble iron (III) salts, water-soluble cobalt (III) salts, water-soluble copper (II) salts, water-soluble quinones, nitrosophenols, complex salts of an organic acid and a polyvalent cation such as iron (III), cobalt (III) or copper (II) (for example, metal complex salts of aminopolycarboxylic acids such as ethylenediaminetetraacetic acid, nitrilotriacetic acid, iminodiacetic acid or N-hydroxyethylethylenediaminetriacetic acid, malonic acid, tartaric acid, malic acid, diglycolic acid, or dithioglycolid acid, 2,6-dipicolinic acid copper complex salt, etc.), peroxy acids such a alkyl peroxy acids, persulfate salts, permanganate salts or hydrogen peroxide, hydrochlorides, chlorine, bromine, etc., are used, either individually or in an appropriate combination. In addition, bleach accelerators as described in US Pat. Nos. 3,042,520 and 3,241,966 can also be employed.

In the fixation step, any known fixing solutions can be used. For example, ammonium thiosulfate, sodium thiosulfate or potassium thiosulfate can be used as a fixing agent in an amount of about 50 to 200 g/litre and, in addition, a stabilizing agent such as sulfite salts or metabisulfite salts, a hardening agent such as potassium alum, a pH buffer such as acetate salts or borate salts, can be present in the fixing solution. The fixing solutions have a pH of about 3 to 12, usually a pH of about 3 to 8.

Suitable bleaching agents, fixing agents and bleach-fix baths are described, e.g., in US 3,582,322.

Image-stabilizing baths can also be employed according to the techniques as described in US Pat. Nos. 2,515,121, 2,518,686 and 3,140,177.

Suitable processing steps as utilizing low replenishment rates in a short latent image time within 12 seconds after exposure of the photographic paper with laser (digital) scanning as described in US 6,949,334 can also be employed.

According to a second aspect of the present invention there is provided a method for preparing a photographic paper comprising applying a composition to a support comprising a base layer and one or more light-sensitive emulsion layers, wherein the composition comprises a hydrophilic colloid binder and colloidal silica in a weight ratio of 0.3:1 to 3:1 (preferably 0.3:1 to 2:1) and the colloidal silica has a mean particle size of 2 to 10 nm.

In this method the composition is preferably applied to the support at a coating speed higher than 200 m/min, more preferably higher than 300m/min.

The composition is preferably applied to the support using a slide coater or curtain coater. In a preferred embodiment the composition and at least one light-sensitive emulsion layer (preferably at least three light-sensitive emulsion layers) are applied to the support simultaneously optionally along with the abovementioned composition.

The composition preferably comprises a liquid medium, a hydrophilic colloid binder and colloidal silica in a weight ratio of 0.3:1 to 3:1 (preferably 0.3:1 to 2:1), wherein the colloidal silica has a mean particle size of 2 to 10 nm. Typical liquid media include water and mixtures comprising water and one or more water-miscible organic solvents.

Preferably the composition has a viscosity at 20°C of 30 to 75cP, more preferably 40 to 60 cP.

In one embodiment the composition further comprises a hardening agent and the hydrophilic colloid binder in a ratio (R) satisfying the following equation: $R = \left(Hmol/HCg\right)$ wherein:
- R: is greater than 0.00013;
- Hmol: is the number of moles of hardening agent in the composition; and
- HCg: is the weight in grams of hydrophilic colloid binder in the composition.

The method preferably further comprises the step of drying the composition after it has been applied to the support.

According to a third aspect of the present invention there is provided an album-book comprising one or more photographs comprising photographic paper according to the present invention.

To make full use of the advantages of the present invention, the album-book preferably comprises at least two of said photographs positioned such that the photographs are in face-to-face contact when the album book is closes. In this way there is no need to include an interleaf foil separating the faces of the photographs.

The invention is further explained by reference to the following non-limiting examples. Unless otherwise indicated herein, all parts, percents, ratios are by weight.

### Examples

A base layer was prepared by subjecting a photographic grade paper coated with a polyethylene resin on both sides to surface corona discharge treatment. The base layer was provided with a gelatin undercoat layer containing sodium dodecylbenzene sulfonate and then successively coated simultaneously, in one step, with all light-sensitive emulsion layers using a slide coater at 300 m/min. This resulted in a color photographic paper having the layer configuration described below:
- Base layer:: Polyethylene (PE) resin-laminated paper; top-side PE 23 g/m²; back-side PE 22 g/m².

The polyethylene resin on the first layer side contained a white pigment (TiO2: content of 16 wt%, ZnO: content of 4 wt%), a fluorescent whitening agent (4,4'-bis(5-methylbenzoxazoryl)stilbene: content 0.03 wt%), and a blue dye (ultramarine blue).

Ratio of the top-side/back side resin weight on the paper is 1.05.

The thickness of the base layer was about 163 micron.

All of the Examples had an identical base layer and first to sixth layers as described below. The outer-most (seventh) layer was varied as described below in order to compare the performance of photographic papers comprising an outer-most layer of the present invention with Comparative photographic papers falling outside of the claims.

The silicas used in the Examples and Comparative Examples were colloidal silicas obtained from H.C. Starck under the trade name Levasil^{™}.

The hardening agent used in the Examples and Comparative Examples is sodium 1-oxy-3,5-dichloro-s-triazine.

The following dyes (coating amounts in brackets) were included in the layers where indicated.

### Layer constitution

The composition of each layer is shown below. The numbers show coating amounts (g/m²). In the case of the silver halide emulsion, the coating amount is in terms of silver.

**First layer (Blue sensitive emulsion layer)**

| Examples and Comparative Examples | Component | Amount |
|---|---|---|
| All | Silver chlorobromoiodide Emulsion A^{#} (containing gold-sulfur sensitized cubic grains and being a 3:7 (by mole on a silver basis) mixture of large-sized Emulsion A-1 and a small-sized Emulsion A-2) | 0.24 |
| | Gelatin | 1.25 |
| | Yellow coupler (Ex Y1) | 0.34 |
| | Color image stabilizer (Cpd-1) | 0.07 |
| | Color image stabilizer (Cpd-2) | 0.04 |
| | Color image stabilizer (Cpd-3) | 0.07 |
| | Color image stabilizer (Cpd-8) | 0.02 |
| | Solvent (Solv-1) | 0.21 |

| | | |
|---|---|---|
| # = Preparation Emulsion A is disclosed on columns 94/95/96 in US Pat No. 6,921,631. | | |

**Second layer (Color Mixing Inhibiting layer)**

| Examples and Comparative Examples | Component | Amount |
|---|---|---|
| All | Gelatin | 1.15 |
| | Color mixing inhibitor (Cpd-4) | 0.10 |
| | Color mixing image stabilizer(Cpd-5) | 0.018 |
| | Color image stabilizer(Cpd-6) | 0.13 |
| | Color image stabilizer (Cpd-7) | 0.07 |
| | Dye-1 | 0.001 |
| | Dye-2 | 0.001 |
| | Dye-3 | 0.0015 |
| | Dye-4 | 0.0035 |
| | Solvent (Solv-1) | 0.04 |
| | Solvent (Solv-2) | 0.12 |
| | Solvent (Solv-5) | 0.11 |
| Ex. 1 to 7 and CE 1 to 8 | Hardening agent | 0.0345 |
| Ex. 8 | Hardening agent | 0.0397 |
| Ex. 9 | Hardening agent | 0.0449 |
| Ex. 10 | Hardening agent | 0.0528 |
| Ex. 11 | Hardening agent | 0.0475 |

**Third layer (Green sensitive emulsion layer)**

| Examples and Comparative Examples | Component | Amount |
|---|---|---|
| All | Silver chlorobromoiodide Emulsion C* 0.14 (containing gold-sulfur sensitized cubic grains and being a 1:3 (by mole on a silver basis) mixture of large-sized Emulsion C-1 and a small-sized Emulsion C-2) | 0.14 |
| | Gelatin | 0.46 |
| | Magenta coupler (Ex M) | 0.15 |
| | Ultraviolet absorber (UV-A) | 0.14 |
| | Color image stabilizer (Cpd-2) | 0.003 |
| | Color image stabilizer (Cpd-5) | 0.002 |
| | Color image stabilizer (Cpd-6) | 0.09 |
| | Color image stabilizer (Cpd-8) | 0.02 |
| | Color image stabilizer (Cpd-9) | 0.01 |
| | Color image stabilizer (Cpd-10) | 0.01 |
| | Color image stabilizer (Cpd-11) | 0.0001 |
| | Solvent (Solv-3) | 0.09 |
| | Solvent (Solv-4) | 0.18 |
| | Solvent (Solv-5) | 0.27 |

| | | |
|---|---|---|
| * = Preparation Emulsion C is disclosed in columns 96/97 in US 6,921,631. | | |

**Fourth layer Color Mixing Inhibiting layer)**

| Examples and Comparative Examples | Component | Amount |
|---|---|---|
| All | Gelatin | 0.68 |
| | Color mixing inhibitor (Cpd-4) | 0.06 |
| | Color image stabilizer (Cpd-5) | 0.011 |
| | Color image stabilizer (Cpd-6) | 0.08 |
| | Color image stabilizer (Cpd-7) | 0.04 |
| | Dye-1 | 0.001 |
| | Dye-2 | 0.001 |
| | Dye-3 | 0.0015 |
| | Dye-4 | 0.0035 |
| | Solvent (Solv-1) | 0.02 |
| | Solvent (Solv-2) | 0.07 |
| | Solvent (Solv-5) | 0.065 |
| Ex. 1 to 7 and CE 1 to 8 | Hardening agent | 0.0115 |
| Ex. 8 | Hardening agent | 0.0132 |
| Ex. 9 | Hardening agent | 0.0150 |
| Ex. 10 | Hardening agent | 0.0176 |
| Ex. 11 | Hardening agent | 0.0158 |

**Fifth layer (Red sensitive emulsion layer)**

| Examples and Comparative Examples | Component | Amount |
|---|---|---|
| All | Silver chlorobromoiodide Emulsion E^{$} (containing gold-sulfur sensitized cubic grains and being a 5:5 (by mole on a silver basis) mixture of large-sized Emulsion E-1 and a small-sized Emulsion E-2) | 0.10 |
| | Gelatin | 1.11 |
| | Cyan coupler (ExC-1) | 0.02 |
| | Cyan coupler (ExC-3) | 0.01 |
| | Cyan coupler (ExC-4) | 0.11 |
| | Cyan coupler (ExC-5) | 0.01 |
| | Color image stabilizer (Cpd-1) | 0.01 |
| | Color image stabilizer (Cpd-6) | 0.06 |
| | Color image stabilizer (Cpd-7) | 0.02 |
| | Color image stabilizer (Cpd-9) | 0.04 |
| | Color image stabilizer (Cpd-10) | 0.01 |
| | Color image stabilizer (Cpd-14) | 0.01 |
| | Color image stabilizer (Cpd-15) | 0.12 |
| | Color image stabilizer (Cpd-16) | 0.01 |
| | Color image stabilizer (Cpd-17) | 0.01 |
| | Color image stabilizer (Cpd-18) | 0.07 |
| | Color image stabilizer (Cpd-20) | 0.01 |
| | Ultraviolet absorber (UV-7) | 0.01 |
| | Solvent (Solv-5) | 0.15 |

| | | |
|---|---|---|
| ^{$}= Preparation Emulsion E is disclosed in columns 97/98 in US 6,921,631. | | |

**Sixth layer (Ultraviolet Absorbing layer)**

| Examples and Comparative Examples | Component | Amount |
|---|---|---|
| | Gelatin | 0.46 |
| | Ultraviolet absorber (UV-B) | 0.35 |
| | Compound (S1-4) | 0.0015 |
| | Solvent (Solv-7) | 0.18 |
| Ex. 1 to 7 and CE 1 to 8 | Hardening agent | 0.0690 |
| Ex. 8 | Hardening agent | 0.0794 |
| Ex. 9 | Hardening agent | 0.0897 |
| Ex. 10 | Hardening agent | 0.1056 |
| Ex. 11 | Hardening agent | 0.0950 |

### Seventh layer (outer-most layer)

Compositions for preparing the outermost layer were prepared by adding the colloidal silicas mentioned in Table 2 to stock solutions comprising the ingredients mentioned in Table 1 and a liquid medium. The compositions were then applied to the sixth layer mentioned above such that the resultant, outer-most layer, after drying, comprised the amounts of hydrophilic colloid binder and colloidal silica indicated in Tables 1 and 2 below (in g/m²). The compositions had a pH of 9.5 at 40°C.

**Table 1**

| Components | Amounts coated A (g/m²) | Amounts coated B (g/m²) | Amounts coated C (g/m²) |
|---|---|---|---|
| Gelatin (Acid processed) (a hydrophilic colloid binder) | 0.86 | 0.86 | 0.29 |
| Acryl-modified copolymer of polyvinyl alcohol (modification degree: 17%) (a hydrophilic colloid binder) | 0.04 | 0.04 | 0.01 |
| Polymethyl methacrylate mean particle size 4 micron | - | 0.01 | 0.01 |
| Surface active agents (Cmp-13) | 0.04 | 0.04 | 0.02 |
| Liquid paraffin | 0.01 | 0.01 | 0.004 |

In stock solutions A and B amounts varying silica was added (in sizes) at 40°C and varying amounts (in g/m²) as shown in Table 2 below.

### Results

The extent to which various photographic papers stick together was evaluated in the two tests described below as the "Blocking Test" or "Peeling Behaviour". The Peeling Behaviour Test was a much more difficult test of sticking performance than the Blocking Test and was designed as a more rigorous test for the best performing non-stick photographic papers. The protocols for performing these tests are described after the results.

In Tables 2 to 4, the values of R refer to the ratio of hardening agent to hydrophilic colloid binder in the photographic paper as a whole.

The Actual Examples are photographic papers according to the present invention whereas the Comparative Examples are not. As described in more detail below, the results are scored from 1 to 5, with 1 being the best score and 5 being the worst score. Two results are given for Ex. 1 to Ex. 6, Ex. 8 to Ex. 10 and CE1 to CE 8 in the tables (e.g. "2/1 "), the first for an outermost layer based on stock solution A and the second for an outermost layer based on stock solution B. Ex. 7 and Ex. 11 were prepared from stock emulsion C.

### Tables 2 and 3 - Blocking Test Results

**Table 2**

| | Actual Examples | | | | | | |
|---|---|---|---|---|---|---|---|
| | Ex. 1 | Ex. 2 | Ex. 3 | Ex. 4 | Ex. 5 | Ex. 6 | Ex. 7 |
| Silica (g/m²) | 0.4 | 0.6 | 1.0 | 0.3 | 0.5 | 0.6 | 0.9 |
| Silica mean particle size (nm) | 9 | 9 | 9 | 6 | 6 | 6 | 6 |
| Weight ratio silica: hydrophilic colloid binder | 0.44 | 0.67 | 1.11 | 0.33 | 0.56 | 0.67 | 3.0 |
| Value of R | 10⁻⁴ | 10⁻⁴ | 10⁻⁴ | 10⁻⁴ | 10⁻⁴ | 10⁻⁴ | 10⁻⁴ |
| Blocking Test Result | 3/3 | 2/2 | 2/1 | 3/2 | 2/1 | 1/1 | 1 |

**Table 3**

| | Comparative Examples | | | | | | | |
|---|---|---|---|---|---|---|---|---|
| | CE 1 | CE 2 | CE 3 | CE 4 | CE 5 | CE 6 | CE 7 | CE 8 |
| Silica (g/m²) | 0.1 | 1.0 | 0.1 | 1.0 | 0.1 | 1.0 | 0.2 | 0.1 |
| Silica mean particle size (nm) | 55 | 55 | 30 | 30 | 15 | 15 | 9 | 6 |
| Weight ratio silica: hydrophilic colloid binder | 0.11 | 1.11 | 0.11 | 1.11 | 0.11 | 1.11 | 0.22 | 0.11 |
| Value of R | 10⁻⁴ | 10⁻⁴ | 10⁻⁴ | 10⁻⁴ | 10⁻⁴ | 10⁻⁴ | 10⁻⁴ | 10⁻⁴ |
| Blocking Test Result | 5/5 | 5/5 | 5/5 | 5/5 | 5/5 | 5/5 | 5/4 | 4/4 |

| | | | | | | | | |
|---|---|---|---|---|---|---|---|---|
| * = colloidal silica from Company H.C. Starck (Trade name Levasil^{™}). Remark: Outer-most layers with silica loads above 1.5 g/m2 could not be coated with coating speeds above 200m/min using a slide coater. | | | | | | | | |

The structural formulae of the compounds used herein are illustrated below:

**Table 4 - Peeling Behaviour Test Results & Variation of R**

| | Actual Examples | | | | | |
|---|---|---|---|---|---|---|
| | Ex. 6 | Ex. 8 | Ex. 9 | Ex. 10 | Ex. 7 | Ex. 11 |
| Silica (g/m²) | 0.6 | 0.6 | 0.6 | 0.6 | 0.9 | 0.9 |
| Silica mean particle size (nm) | 6 | 6 | 6 | 6 | 6 | 6 |
| Weight ratio silica: hydrophilic colloid binder | 0.67 | 0.67 | 0.67 | 0.67 | 3.0 | 3.0 |
| Value of R | 10⁻⁴ | 0.000115 | 0.000131 | 0.000156 | 10⁻⁴ | 0.000156 |
| Peeling Behaviour Test Result | 5/5 | 4/4 | 3/2 | 2/1 | 5 | 2 |

(ExY-1): Yellow coupler (ExM) Magenta Coupler
40:40:20 (by mole) mixture of (1), (2) and (3):

| | |
|---|---|
| (1) | (2) |
| | |
| (3) | |
| | |
| (ExC-1) Cvan coupler | (Cpd-1) |
| | |
| (ExC-3) Cyan coupler | (ExC-4) Cyan coupler |
| | |
| (ExC-5) Cyan coupler | (Cpd-1) Color image stabiliser |
| | |

| | |
|---|---|
| (Cpd-3) Color image stabilizer | (Cpd-8) Color image stabilizer |
| | |
| n = 7-8 (on average) | |
| (Cpd-4) Color mixing inhibitor | (Cpd-9) Color image stabilizer |
| | |
| (Cpd-5) Color image stabilizer | (Cpd-10) Color image stabilizer |
| | |
| (Cpd-6) Color image stabilizer | (Cpd-11) |
| | |
| number average molecular weight: 600 m/n = 10.90 | |
| (Cpd-7) Color image stabilizer | |
| | |
| (Cpd-13) | (Cpd-18) |
| 7.3 (by mole) mixture of | |
| | |
| and | (Cpd-20) |
| | |
| (Cpd-14) | (Solv-1) |
| | |
| (Cpd-15) | |
| | (Solv-2) |
| (Cpd-16) | |
| | (Solv-4) |
| (Cpd-17) | |
| | (Solv-4) |
| | O = P(OC₆H₁₃(a))₃ |
| (Solv-5) | (UV-5) Ultraviolet absorbent |
| | |
| (Solv-7) | (UV-6) Ultraviolet absorbent |
| | |
| (S1-4) | (UV-7) Ultraviolet absorbent |
| | |
| (UV-1) Ultraviolet absorbent | UV-A: 7:2:2 (by weight) mixture of UV-1, UV-2 and UV-3 |
| | UV-B: 13:3:3:5:3 (by weight) mixture of UV-1, UV-2, UV-3, UV-5 and UV-6 |
| (UV-2) Ultraviolet absorbent | UV-C: 9:1 (by weight) mixture of UV-1 and UV-3 |
| | |
| (UV-3) Ultraviolet absorbent | |
| | |

### Protocols for the Blocking Test and Peeling Behaviour Test

The photographic papers described above were prepared and then aged by storing at 25°C and 60% relative humidity for one week. The resultant papers were then subjected to black development (via daylight exposure) using the following processing and development steps.

### Processing steps:

| | |
|---|---|
| Development: | 45 seconds |
| Fixation: | 45 seconds |
| Washing: | 45 seconds |

### Developer composition:

Fuji Hunt CPRA-pro developer (commercially available).

### Blocking Test:

The developed photographic paper samples were each cut into 3.5 cm by 3.5 cm squares and two samples of each composition were placed on each other (face-to-face). On top of that a weight of 200 g was placed. The samples were stored for 24 hours in a conditioned room at 52°C and 85% relative humidity.

The samples were then put for 1 hour in a conditioned room at 25°C and 60% relative humidity. From these samples the blocking (i.e. the extent to which the samples stuck together) was evaluated by the following procedure. The two parts of each sample were pulled apart and the level of damage to the faces was evaluated. The following classification was used and two scores were given (e.g. 1/1), the first for the outermost layer derived from stock solution A, and the second for the outermost layer derived from stock solution B. When only one score is provided the outer-most layer was derived from stock solution C:
5: Severe damage: Base layer was completely torn; very poor.
4: Damage: About 50% of photographic paper was torn and emulsion layers damaged; poor.
3: Minor damage + emulsion layers damaged visible by eye; just acceptable.
2: Minor emulsion damage (top-side layer damaged; only visible by microscope); good.
1: No damage; very good.

### Peeling Behaviour Test

The Peeling Behaviour Test was a much more difficult test than the Blocking Test.

The developed photographic paper samples were each cut into 3.5 cm by 3.5 cm squares. Deionised water (20µl) was dropped onto the face of one sample and then the two samples were placed on each other (face-to-face). On top of that a weight of 200 g was placed for 30 seconds and than the two samples were pulled apart and the level of damage to the faces was evaluated. The following classification was used and two scores were given (e.g. 1/1), the first for the outermost layer derived from stock solution A, and the second for the outermost layer derived from stock solution B: When only one score is provided the outer-most layer was derived from stock solution C:
5: Severe damage: Base layer was completely torn.
4: Damage: About 50% of photographic paper was torn and emulsion layers damaged.
3: Minor damage + emulsion layers damaged visible by eye.
2: Minor emulsion damage (top-side layer damaged; only visible by microscope).
1: No damage.

## Claims

1. An album-book comprising at least two photographs positioned such that the photographs are in face-to-face contact when the album book is closed, wherein said photographs comprise photographic paper comprising an outer-most layer comprising a hydrophilic colloid binder and colloidal silica, wherein:
(i) the weight ratio of colloidal silica to hydrophilic colloid binder in said layer is 0.3:1 to 3:1; and
(ii) the colloidal silica has a mean particle size of 2 to 10 nm.

2. An album-book according to claim 1 wherein there is no interleaf foil separating the faces of said photographs.

3. An album-book according to claim 1 or 2 wherein the outer-most layer comprises 0.3 to 1.5 g/m² of the colloidal silica.

4. An album-book according to any one of the preceding claims wherein the colloidal silica has a mean particle size of 3 to 9 nm.

5. An album-book according to any one of the preceding claims wherein the photographic paper comprises a base layer comprising paper.

6. An album-book according to any one of the preceding claims which comprises a base layer comprising a resin coated paper having a thickness of 100 to 250 micrometres.

7. An album-book according to any one of the preceding claims wherein the photographic paper comprises a base layer comprising a paper having a top-side resin and a back-side resin in a weight ratio of 0.7:1 to 1.3.1.

8. An album-book according to any one of the preceding claims wherein the photographic paper further comprises a hardening agent and the ratio (R) of hardening agent to hydrophilic colloid binder satisfies the following equation: $R = \left(Hmol/HCg\right)$
wherein:
R is greater than 0.00013;
Hmol is the number of moles of hardening agent; and
HCg is the weight in grams of hydrophilic colloid binder.

9. An album-book according to any one of the preceding claims wherein the hydrophilic colloid binder is a gelatin.

10. Use of photographic paper to make an album-book comprising at least two photographs positioned such that the photographs are in face-to-face contact when the album book is closed, wherein said photographic paper comprises an outer-most layer comprising a hydrophilic colloid binder and colloidal silica, wherein:
(i) the weight ratio of colloidal silica to hydrophilic colloid binder in said layer is 0.3:1 to 3:1; and
(ii) the colloidal silica has a mean particle size of 2 to 10 nm.

11. The use according to claim 10 wherein there is no interleaf foil separating the faces of the photographs.

## Patentansprüche

1. Albumbuch, umfassend wenigstens zwei Photographien, die so angeordnet sind, dass die Photographien von Vorderseite zu Vorderseite in Kontakt stehen, wenn das Albumbuch geschlossen ist, wobei die Photographien photographisches Papier umfassen, das eine Äußerste Schicht umfasst, die ein hydrophiles Kolloidbindemittel und kolloidales Siliciumoxid umfasst, wobei:
(i) das GewichtsverhÄltnis von kolloidalem Siliciumoxid zu hydrophilem Kolloidbindemittel in der Schicht 0,3:1 bis 3:1 betrÄgt; und
(ii) das kolloidale Siliciumoxid eine mittlere Partikelgröße von 2 bis 10 nm aufweist.

2. Albumbuch gemÄß Anspruch 1, wobei kein Zwischenblatt vorhanden ist, das die Vorderseiten der Photographien trennt.

3. Albumbuch gemÄß Anspruch 1 oder 2, wobei die Äußerste Schicht 0,3 bis 1,5 g/m² des kolloidalen Siliciumoxids umfasst.

4. Albumbuch gemÄß einem der vorstehenden Ansprüche, wobei das kolloidale Siliciumoxid eine mittlere Partikelgröße von 3 bis 9 nm aufweist.

5. Albumbuch gemÄß einem der vorstehenden Ansprüche, wobei das photographische Papier eine TrÄgerschicht umfasst, die Papier umfasst.

6. Albumbuch gemÄß einem der vorstehenden Ansprüche, die eine TrÄgerschicht umfasst, die ein harzbeschichtetes Papier mit einer Dicke von 100 bis 250 Mikrometer umfasst.

7. Albumbuch gemÄß einem der vorstehenden Ansprüche, wobei das photographische Papier eine TrÄgerschicht umfasst, die Papier mit einem Vorderseitenharz und einem Rückseitenharz in einem GewichtverhÄltnis von 0,7:1 bis 1,3:1 umfasst.

8. Albumbuch gemÄß einem der vorstehenden Ansprüche, wobei das photographische Papier ferner ein HÄrtungsmittel umfasst und das VerhÄltnis (R) von HÄrtungsmittel zu hydrophilem Kolloidbindemittel folgende Gleichung erfüllt: $R = \left(Hmol/HCg\right)$
wobei:
R größer als 0,00013 ist;
Hmol die Anzahl der Mol an HÄrtungsmittel ist; und
HCg das Gewicht des hydrophilen Kolloidbindemittels in Gramm ist.

9. Albumbuch gemÄß einem der vorstehenden Ansprüche, wobei das hydrophile Kolloidbindemittel Gelatine ist.

10. Verwendung von photographischem Papier zum Herstellen eines Albumbuchs, das wenigstens zwei Photographien umfasst, die so angeordnet sind, dass die Photographien von Vorderseite zu Vorderseite in Kontakt stehen, wenn das Albumbuch geschlossen ist, wobei das photographische Papier eine Äußerste Schicht umfasst, die ein hydrophiles Kolloidbindemittel und kolloidales Siliciumoxid umfasst, wobei:
(i) das GewichtsverhÄltnis von kolloidalem Siliciumoxid zu hydrophilem Kolloidbindemittel in der Schicht 0,3:1 bis 3:1 betrÄgt; und
(ii) das kolloidale Siliciumoxid eine mittlere Partikelgröße von 2 bis 10 nm aufweist.

11. Verwendung gemÄß Anspruch 10, wobei kein Zwischenblatt vorhanden ist, das die Vorderseiten der Photographien trennt.

## Revendications

1. Livre-album comprenant au moins deux photographies positionnées de telle sorte que les photographies sont en contact face-à-face lorsque le livre-album est fermé, lesdites photographies comprenant du papier photographique comprenant une couche la plus à l'extérieur comprenant un liant colloïdal hydrophile et de la silice colloïdale :
(i) le rapport pondéral de la silice colloïdale au liant colloïdal hydrophile dans ladite couche étant de 0,3:1 à 3:1 ; et
(ii) la silice colloïdale possédant une taille moyenne de particules de 2 à 10 nm.

2. Livre-album selon la revendication 1, dans lequel il n'y a pas de feuillet intercalaire séparant les faces desdites photographies.

3. Livre-album selon la revendication 1 ou la revendication 2, dans lequel la couche la plus à l'extérieur comprend de 0,3 à 1,5 g/m² de silice colloïdale.

4. Livre-album selon l'une quelconque des revendications précédentes, dans lequel la silice colloïdale possède une taille moyenne de particules de 3 à 9 nm.

5. Livre-album selon l'une quelconque des revendications précédentes, dans lequel le papier photographique comprend une couche de base comprenant du papier.

6. Livre-album selon l'une quelconque des revendications précédentes qui comprend une couche de base comprenant un papier recouvert de résine possédant une épaisseur de 100 à 250 micromètres.

7. Livre-album selon l'une quelconque des revendications précédentes, dans lequel le papier photographique comprend une couche de base comprenant un papier possédant une résine sur la face supérieure et une résine sur la face arrière dans un rapport pondéral de 0,7:1 à 1,3:1.

8. Livre-album selon l'une quelconque des revendications précédentes, dans lequel le papier photographique comprend en outre un agent durcisseur et le rapport (R) de l'agent durcisseur au liant colloïdal hydrophile satisfait l'équation suivante : $R = \left(Hmol/HCg\right)$
dans laquelle :
R est supérieur à 0,00013 ;
Hmol représente le nombre de moles de l'agent durcisseur ; et
HCg représente le poids en grammes du liant colloïdal hydrophile.

9. Livre-album selon l'une quelconque des revendications précédentes, dans lequel le liant colloïdal hydrophile est une gélatine.

10. Utilisation de papier photographique pour faire un livre-album comprenant au moins deux photographies positionnées de telle sorte que les photographies sont en contact face-à-face lorsque le livre-album est fermé, ledit papier photographique comprenant une couche la plus à l'extérieur comprenant un liant colloïdal hydrophile et de la silice colloïdale :
(i) le rapport pondéral de la silice colloïdale au liant colloïdal hydrophile dans ladite couche étant de 0,3:1 à 3:1 ; et
(ii) la silice colloïdale possédant une taille moyenne de particules de 2 à 10 nm.

11. Utilisation selon la revendication 10, dans laquelle il n'y a pas de feuillet intercalaire séparant les faces desdites photographies.
